

3,702,248

## BLEACH-FIX ADDITIVES

David Gerald Alcock, John Colin Brown, Enzo Piccotti, and Norman John Lungius, Ilford, England, assignors to Ilford Limited, Ilford, Essex, England  
No Drawing. Filed Dec. 22, 1970, Ser. No. 100,839  
Claims priority, application Great Britain, Dec. 23, 1969, 62,680/69

Int. Cl. G03c 7/16

U.S. Cl. 96—22

14 Claims

### ABSTRACT OF THE DISCLOSURE

This application describes a bleach-fix bath for use in processing colour photographic material comprising a mild oxidising agent, a silver-halide solvent and a bleach-fix accelerator which is a water soluble selenium compound selected from defined classes of selenosemi-carbazides and analogous bis-compounds, 1,2,4-triazole-3-selenols and 5,5-bis, 1,2,4-triazole-3-selenols, the invention including the baths per se and their use in colour processing of photographic material.

This invention relates to the processing of photographic material comprising silver halide emulsion layers to yield material having colour dye images therein.

In the processing of conventional colour photographic material a developable silver salt image is developed with an aromatic primary amino developing agent of the para-phenylene diamine type (a so-called "colour developer") in the presence of a compound (a so-called "colour coupler") which will combine with the oxidation products of the colour developer to form an azomethine or quinone-imine dye. The dye is thus formed in situ with the developed silver image. Subsequently the product must be treated with a bleach bath and a fixing bath or a combined bleach-fix bath thereby to remove silver and any residual silver halide or other silver salt, leaving in the product only the dye image.

In the silver-dye-bleach process of colour photography the photographic material comprises at least one silver halide emulsion layer which includes as a dispersion therein an organic dyestuff of the type which can be destroyed (or bleached) by finely divided silver in a suitable treatment bath. The organic dyestuff is usually an azo dye. Most commonly three such silver halide emulsion layers are present each of which is sensitive to a different region of the visible spectrum and each of which contains a different azo dye. The usual processing sequence for the production of a dye image in the material is after an imagewise exposure to develop the material in a black and white developer. The development is then stopped and the unexposed silver halide is fixed out. Then after washing the material is treated in a dye-bleach bath which oxidises the silver image and simultaneously reduces (bleaches) the dye in the region of the silver image. The silver salts and any residual silver must then be removed. This is usually accomplished by washing the material after its treatment in the dye-bleach bath and then treating it in a bleach bath followed by a fixing bath or treating it in a combined bleach-fix bath. The photographic material then contains a dye image only; this dye image being usually a direct positive reproduction of the original.

In one commercially available silver-dye-bleach material the amount of residual silver left after the dye-bleach step is not negligible because this material requires to be processed so that the dye-bleach step is terminated before all the image silver has been used in reducing the dye. Thus in the processing of this silver-dye-bleach material

in particular it is essential that an effective silver bleach step succeeds the dye-bleach step in order to ensure that the residual silver is removed as completely as possible from the material.

5 In both the processing of conventional colour photographic material and in the processing of silver-dye-bleach material the use of a combined bleach-fix bath is preferable because it results in a reduction of the processing time and of the cost of processing equipment required. 10 Normally a bleach-fix bath comprises a mild oxidising agent for example a ferric chelate complex, a cupric complex, a salt or a cobalt (III) complex together with a silver halide solvent or fixing agent for example a water-soluble thiosulphate or a water-soluble thiocyanate. Strong oxidising agents cannot be used because they tend to oxidise the silver halide solvent.

15 Stable bleach-fix solutions comprising ferric chelate complexes and sodium thiosulphate may be obtained but because of the weak oxidising power of the ferric chelate complex such bleach-fix bath can only be used commercially for the processing of photographic materials with a fairly low silver content.

20 According to the present invention in the processing of photographic material comprising silver halide emulsion layers to yield material having colour dye images therein there is provided a bleach-fix step which comprises treating the photographic material with a stable bleach-fix bath which comprises an aqueous solution of a mild oxidising agent and a silver halide solvent which is either a 25 water-soluble thiosulphate or a water-soluble thiocyanate in the presence of a bleach-fix accelerator which is selected from (a) a water-soluble selenosemi-carbazide of the general Formula I:



30 wherein one of  $\text{R}_1$  and  $\text{R}_2$  is a hydrogen atom or an alkyl, aralkyl or aryl group or a group  $\text{R}_6\text{CO}-$  where  $\text{R}_6$  is a hydrogen atom or an alkyl, alkoxy or heterocyclic group, or a group  $\text{NR}_7\text{R}_8-\text{CSe}-$  where  $\text{R}_7$  and  $\text{R}_8$  are each hydrogen atoms or alkyl groups and the other of  $\text{R}_1$  and  $\text{R}_2$  is a hydrogen atom or an alkyl group,  $\text{R}_3$  is a hydrogen atom or an alkyl, aralkyl or aryl group, one of  $\text{R}_4$  and  $\text{R}_5$  is a hydrogen atom or an alkyl, aralkyl or aryl group and the other of  $\text{R}_4$  and  $\text{R}_5$  is a hydrogen atom or an alkyl group but at least one of  $\text{R}_3$ ,  $\text{R}_4$  or  $\text{R}_5$  being a hydrogen atom and there being not more than one group selected from aryl, aralkyl and heterocyclic present in the compound or (b) a water-soluble compound of the general Formula II:



35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865

nol wherein the triazole rings are linked directly or via a link



wherein  $n$  is 1-4 and wherein one nitrogen atom in each of the triazole rings carries a substituent selected from a hydrogen atom and an alkyl, aryl and aralkyl group.

It is to be understood that the triazole-selenol compounds of (c) and (d) above have been defined with reference to their selenol form but these compounds may be present in their tautomeric selenone form in which case there is an additional substituent hydrogen atom in the ring or rings.

The preferred compounds for use in the present invention are those of Formula I wherein each of  $R_1$ - $R_6$  are hydrogen atoms or alkyl groups. Other preferred compounds are those of Formula II wherein each of  $R_9$ - $R_{16}$  is a hydrogen atom. The preferred triazole-selenols of (c) are those wherein the 5-carbon atom carries an alkyl or hydroxy group and one of the nitrogen atoms carries a substituent hydrogen atom. The preferred bis-triazole-selenols of (d) are those wherein one nitrogen atom in each of the triazole rings carries a substituent hydrogen atom.

By "stable bleach-fix bath which comprises an aqueous solution of a mild oxidising agent and a silver halide solvent" is meant a bleach-fix bath wherein the oxidising agent is strong enough to bleach the silver but is not strong enough to oxidise the silver halide solvent, i.e. the thiocyanate or the thiosulphate, to an appreciable degree.

The preferred mild oxidising agents for use in the present invention are ferric chelate complexes or diaquo-tetramminecobalt (III) complexes.

By ferric chelate complex is meant a co-ordination compound of the ferric ion and a compound which comprises nitrogen and/or oxygen-containing co-ordinating groups. The most important co-ordinating groups are amino, heterocyclic nitrogen, carboxyl and carbonyl groups.

The preferred ferric chelate complex for use in the bleach-fix step of the present invention is a ferric ethylenediamine-tetraacetic acid complex. It is to be understood that this compound may be used as such in the preparation of a bleach-fix bath or it may be formed in situ in a bleach-fix bath by ethylenediaminetetraacetic acid reacting with a ferric salt e.g. ferric chloride. In the examples which follow the ferric ethylenediaminetetraacetic acid complex has been formed in situ.

Other ferric chelate complexes which may be used in the present invention are for example pyridine-2:6-dicarboxylateferrate (III) complex, iminodiacetatoferate (III) complex and nitrilo-triacetate-ferrate (III) complex.

The selenosemicarbazides of the above Formula I are known compounds as shown by the references set forth below.

The following Formula III indicates the nitrogen atom referred to in the references.



4-phenylselenosemicarbazide—preparation described by Jensen and Frederiksen, Z. anorg. allgem. Chem. 230, 31-3 (1936)

2-phenylselenosemicarbazide—preparation described by Mautner and Kumler, J. Amer. Chem. Soc. 97-101 (1956)

4-ethylselenosemicarbazide—preparation described by Huls and Renson, Bull. soc. chim. Belges 65, 684-95 (1956)

4-propylselenosemicarbazide—preparation described by M. Colland-Charon, Huls and Renson, Bull. soc. chim. Belges 71, 541-53 (1962)

preparations described by Colland-Charon, Huls and Renson, Bull. soc. chim., Belges 71, 554-62 (1962):

1-phenylselenosemicarbazide, and  
1-(p-tolyl) selenosemicarbazide

preparations described by Jensen, Felbert, Pedersen and Svaholm, Acta chem. Scand. 20 (1) 278-81 (1966):



10 preparations described by Bulka, Ahlens and Tucek, Chem. Ber. 100 (4) 1373-8 (1967):  
2-methyl-4-phenylselenosemicarbazide  
4-(p-chlorophenyl)selenosemicarbazide and  
4-(p-methoxyphenyl)selenosemicarbazide

15 20 15 However compounds of Formula I wherein  $R_1$  is a group  $R_5 \text{CO}-$ , i.e. the monocyl derivatives of the selenosemicarbazides may be prepared by reacting an equimolecular amount of a selenosemicarbazide with an acylating agent, for example an acid chloride or an acid anhydride; the reaction usually being carried out in an organic solvent at a low temperature.

The compounds of Formula I wherein one of  $R_1$  and  $R_2$  is a group  $\text{NR}_7\text{R}_8-\text{CSe}-$  where  $\text{R}$  and  $\text{R}_8$  are each hydrogen atoms or alkyl groups may be prepared by reacting a compound of the general Formula IV:



30 where  $\text{R}_4$  and  $\text{R}_5$  have the meanings assigned to them in Formula I, with hydrogen selenide.

The compounds of Formula II may be prepared by reacting a selenosemicarbazide with a dibasic acid chloride; the reaction usually being carried out in an organic solvent at a low temperature.

35 40 The production of the 1,2,4-triazole-3-selenols of (c) wherein there is attached to the 5-carbon atom an alkyl, group comprises reacting a selenosemicarbazide of the general Formula V:



45 wherein each of  $\text{R}_{24}$ ,  $\text{R}_{25}$ , and  $\text{R}_{26}$  is a hydrogen atom or two of them are hydrogen atoms and one of them is a group selected from alkyl, aryl and aralkyl, with an acid chloride of the general formula  $\text{R}_{21}\text{COCl}$  in the presence of a base or with an acid anhydride of the general formula

50  $\text{R}_{21}\text{COOR}_{21}$  wherein  $\text{R}_{21}$  is an alkyl group and then ring closing this acyl derivative by heating it in the presence of an alkali metal salt of a weak acid for example an acetate or carbonate, or in the presence of an alkali metal hydroxide or an alkoxide.

55 The production of the 1,2,4-triazole-3-selenols of (c) wherein there is attached to the 5-carbon atom a hydrogen atom or an alkyl group which comprises from 1 to 4 carbon atoms comprises reacting a selenosemicarbazide of the above general Formula V with a carboxylic acid of

60 the general formula  $\text{R}_{27}\text{COOH}$  where  $\text{R}_{27}$  is a hydrogen atom or an alkyl group having 1 to 4 carbon atoms, to form the acyl derivative of the selenosemicarbazide, and then ring closing this acyl derivative by heating it in the presence of an alkali metal salt of a weak acid, for example an acetate or carbonate, or in the presence of an alkali metal hydroxide or an alkoxide.

The production of the 1,2,4-triazole-3-selenols of (c) wherein there is attached to the 5-carbon atom an hydroxy group comprises reacting a selenosemicarbazide of the above Formula V with an alkoxy-, aryloxy- or aralkyloxy-haloformate in the presence of a base to form the alkoxy-, aryloxy- or aralkoxycarbonyl derivative of the selenosemicarbazide and ring closing this compound in the presence of an alkali metal salt of a weak acid or

75 in the presence of an alkali metal hydroxide or alkoxide,

with the elimination of the appropriate alcohol or phenol.

The production of the 1,2,4-triazole-3-selenols of (c) wherein there is attached to the 5-carbon atom an amino, alkylamino, arylamino or aralkylamino group comprises reacting a selenosemicarbazide of the general Formula VI:



wherein  $\text{R}_{37}$  is a hydrogen atom or an alkyl, aryl or aralkyl group and each of  $\text{R}_{38}$ ,  $\text{R}_{39}$ , and  $\text{R}_{40}$  is a hydrogen atom or two of them are hydrogen atoms and the third is a group selected from alkyl, aryl and aralkyl, with an alkali metal hydroxide to effect ring closure and separating the desired product.

Selenosemicarbazides of general Formula VI may be prepared by reacting a bis-selenourea with a one molecular proportion of a methylating agent in a basic medium.

The production of the bis-1,2,4-triazole-selenols may be effected by reacting a selenosemicarbazide with a dibasic acid chloride in the presence of a base to form the acyl derivative and then ring closing the acyl derivative by heating it in a basic medium e.g. in the presence of an alkali metal carbonate, hydroxide or ethoxide.

The bleach-fix accelerators of use in the present invention are preferably added to the bleach-fix bath but they may be present during the bleach-fixing treatment adsorbed to or absorbed in the colour photographic material. In the processing of conventional colour photographic material, i.e. colour negative or colour reversal material bleach-fix accelerators of use in the present invention may be present in any treatment bath or wash bath which is used in the colour development process between the development step and the bleach-fix step. Exemplary of such baths are stop baths and stop-fix baths. The bleach-fix accelerators should not be present, however, in the developing solution as they interfere with the development of the colour material. For the same reason the bleach-fix accelerators of use in the present invention should not be present initially in the photographic material.

In the processing of silver-dye-bleach material the bleach-fix accelerators may be present in the wash bath which succeeds the dye-bleach treatment bath and precedes the bleach-fix bath but the bleach-fix accelerators should not be present during the dye-bleach treatment as they can interfere with this treatment step. Thus the bleach-fix accelerators should not be present initially in the silver-dye-bleach photographic material.

According to another embodiment of the present invention there is provided a stable-bleach-fix bath which comprises an aqueous solution of a mild oxidising agent, as hereinbefore defined, a silver halide solvent which is either a water-soluble thiosulphate or a water-soluble thiocyanate and a bleach-fix accelerator which is either a selenosemicarbazide of the above Formula I or a compound of the above Formula II, or a 1,2,4-triazole-3-selenol of the type (c) as hereinbefore defined, or a bis-1,2,4-triazole-3-selenol of the type (d) as hereinbefore defined.

Preferably in this aspect of the invention the mild oxidising agent is a ferric chelate complex or a diaqua-tetrammine-cobalt (III) complex.

It is preferred that the concentration of the bleach-fix accelerators of the type (a), (b), (c) or (d) as hereinbefore defined present in the bleach-fix bath is greater than 1 mg. per litre of bleach-fix bath. The most preferred

amount being 100 mg. of bleach-fix accelerator per litre of bleach-fix bath.

It is preferred that the concentration of the bleach-fix accelerators of the type (a), (b), (c) or (d) as hereinbefore defined present in a stop bath or a stop-fix bath or in a wash bath is greater than 1 mg. per litre of the solution.

The following examples will serve to illustrate the invention.

In the examples which follow the following bleach-fix accelerators were used:

- (1) 3-selenosemicarbazide
- (2) 1-formyl-3-selenosemicarbazide
- (3) 1-acetyl-3-selenosemicarbazide
- (4) 1-propionyl-3-selenosemicarbazide
- (5) 2-methyl-3-selenosemicarbazide
- (6) 4-methyl-3-selenosemicarbazide
- (7) 1,1'-dimethyl-3-selenosemicarbazide
- (8) 1,2-dimethyl-3-selenosemicarbazide
- (9) 1,2,4-trimethyl-3-selenosemicarbazide
- (10) 1,1',4-trimethyl-3-selenosemicarbazide
- (11) 1-acetyl-4-methyl-3-selenosemicarbazide
- (12) 1-acetyl-4-benzyl-3-selenosemicarbazide
- (13) 4-benzyl-3-selenosemicarbazide
- (14) 1-phenyl-3-selenosemicarbazide
- (15) 2-phenyl-3-selenosemicarbazide
- (16) 4-phenyl-3-selenosemicarbazide
- (17) 2-methyl-4-phenyl-3-selenosemicarbazide
- (18) 1-(2-furoyl)-3-selenosemicarbazide
- (19) 1,1'-oxalyl-bis (3-selenosemicarbazide)
- (20) 1,2,4-triazole-3-selenol
- (21) 5-methyl-1,2,4-triazole-3-selenol
- (22) 4,5-dimethyl-1,2,4-triazole-3-selenol
- (23) 5,5'-bis (1,2,4-triazole-3-selenol)
- (24) 5,5'-methylene-bis(1,2,4-triazole-3-selenol)
- (25) 5,5'-ethylene-bis (1,2,4-triazole-3-selenol)
- (26) 1-ethoxycarbonyl-3-selenosemicarbazide

In the examples which follow a colour negative film was used which was made up as follows:

| Layer order and sensitivity:  | Silver coating weight in mg. of Ag/decimetre <sup>2</sup> |
|-------------------------------|-----------------------------------------------------------|
| Nonstress                     | 13.4                                                      |
| Blue sensitive                | 13.4                                                      |
| Colloidal silver filler layer | 13.1                                                      |
| Green sensitive topcoat       | 13.1                                                      |
| Intralayer                    | 16.0                                                      |
| Green sensitive subcoat       | 16.0                                                      |
| Interlayer                    | 17.5                                                      |
| Red sensitive topcoat         | 13.6                                                      |
| Red sensitive subcoat         | 13.6                                                      |
| Base of cellulose triacetate  | 73.6                                                      |
| Total                         | 73.6                                                      |

In this film:

the blue sensitive layer contained yellow colour coupler of the formula:



the green sensitive layers each contained a magenta colour coupler of the formula:



the red sensitive layers each contained a cyan colour coupler of the formula:



The following processing solutions were used in Examples 1-4

#### STOP-FIX

|                                  |    |      |
|----------------------------------|----|------|
| Sodium thiosulphate pentahydrate | g  | 171  |
| Sodium acetate anhydrous         | g  | 31.4 |
| Sodium sulphite anhydrous        | g  | 4.3  |
| Acetic acid glacial              | ml | 35   |
| Potassium alum                   | g  | 17.0 |
| Ammonium chloride                | g  | 43   |
| Water to 1 litre.                |    |      |

#### BLEACH-FIX

|                                                   |    |      |
|---------------------------------------------------|----|------|
| Disodium tetraborate decahydrate                  | g  | 12.5 |
| Boric acid                                        | g  | 22.5 |
| Sodium hydroxide                                  | g  | 10.0 |
| Ethylenediamine tetraacetic acid                  | g  | 16.2 |
| Disodium salt of ethylenediamine tetraacetic acid | g  | 3.5  |
| Ferric chloride (60% w/v. solution)               | ml | 15.0 |
| Sodium thiosulphate pentahydrate                  | g  | 95   |
| Sodium sulphite anhydrous                         | g  | 4.0  |
| Water to 1 litre.                                 |    | 35   |

#### CONDITIONER

|                                                    |    |      |
|----------------------------------------------------|----|------|
| Disodium salt of ethylene diamine tetraacetic acid | g  | 0.50 |
| Sodium carbonate anhydrous                         | g  | 4.5  |
| Formaldehyde (40% w/v. solution)                   | ml | 10   |
| Lissapol N (8% w/v. solution)                      | ml | 1.7  |
| Water to 1 litre.                                  |    |      |

All processing solutions and wash water were used at 75° F.

The constitution of the colour developing solutions used in the following examples was as follows:

#### COLOUR DEVELOPER A

|                                                             |      |    |
|-------------------------------------------------------------|------|----|
| G.                                                          |      |    |
| Sodium metaborate                                           | 53.3 |    |
| Sodium hydroxide                                            | 2.0  |    |
| Sodium sulphite anhydrous                                   | 3.9  | 55 |
| Potassium bromide                                           | 0.70 |    |
| Hydroxylamine sulphate                                      | 2.34 |    |
| Sodium sulphate anhydrous                                   | 7.8  |    |
| 4-amino-N-ethyl-N-( $\beta$ -hydroxyethyl)-aniline sulphate | 6.0  | 60 |
| Water to 1 litre.                                           |      |    |

#### COLOUR DEVELOPER B

|                                                             |     |  |
|-------------------------------------------------------------|-----|--|
| G.                                                          |     |  |
| Sodium metaborate                                           | 80  |  |
| Sodium sulphite anhydrous                                   | 2.0 |  |
| Potassium bromide                                           | 1.0 |  |
| Hydroxylamine sulphate                                      | 2.6 |  |
| 4-amino-N-ethyl-N-( $\beta$ -hydroxyethyl)-aniline sulphate | 4.6 |  |
| Water to 1 litre.                                           |     |  |

#### EXAMPLES

Pieces of the colour negative film were fogged and processed in a number of processing sequences all containing the use of a bleach-fix bath. The metallic silver remaining

75

in the film at the end of each processing sequence was measured by analysis and expressed in mg. of Ag/decimetre<sup>2</sup>.

When the bleach-fix bath or stop-fix bath contained one of the specified bleach-fix accelerators a reduction in the amount of residual silver resulted. In the examples the residual silver resulting when one of the accelerators was used is expressed as a percentage of that obtained when no accelerator was used (referred to as the control).

10

#### Example 1

Pieces of the colour negative film were processed as follows:

|             |                    | Minutes |
|-------------|--------------------|---------|
| 15          | Colour developer B | 10      |
| Stop-fix    |                    | 14      |
| Wash        |                    | 4       |
| Bleach-fix  |                    | 6       |
| Wash        |                    | 4       |
| Conditioner |                    | 4       |
| Wash        |                    | 4       |
| Dry.        |                    |         |

<sup>1</sup> With and without accelerator.

The silver content of the pieces of film was analysed with the following results:

TABLE 1

| Accelerator compound No. | Concentration of accelerator in the stop-fix bath, mg./dm. <sup>3</sup> | Residual silver mg./dm. <sup>2</sup> | Percent of control |
|--------------------------|-------------------------------------------------------------------------|--------------------------------------|--------------------|
| 1<br>No accelerator      | 300                                                                     | 1.0                                  | 8.4                |
| 100                      | 11.96                                                                   |                                      | 100                |

#### Example 2

Pieces of the colour negative film were processed as follows:

|                    |  | Minutes |
|--------------------|--|---------|
| Colour developer B |  | 10      |
| Stop-fix           |  | 14      |
| Wash               |  | 4       |
| Bleach-fix         |  | 6       |
| 45 Conditioner     |  | 4       |
| Wash               |  | 4       |
| Dry.               |  |         |

<sup>1</sup> With and without accelerator.

The silver content of the pieces of film was analysed with the following results:

TABLE 2

| Accelerator compound No. | Concentration of accelerator in stop-fix bath, mg./dm. <sup>3</sup> | Residual silver as percent of control |
|--------------------------|---------------------------------------------------------------------|---------------------------------------|
| 1                        | 300                                                                 | 10.9                                  |
| 21                       | 300                                                                 | 17.4                                  |

#### Example 3

Pieces of the colour negative film were processed as follows:

|                       |  | Minutes |
|-----------------------|--|---------|
| 65 Colour developer A |  | 6       |
| Stop-fix              |  | 4       |
| Wash                  |  | 4       |
| 70 Wash               |  | 4       |
| Bleach-fix            |  | 16      |
| Conditioner           |  | 4       |
| Wash                  |  | 4       |
| Dry.                  |  |         |

<sup>1</sup> With and without accelerator.

The silver content of the pieces of film was analysed with the following results:

TABLE 3

| Accelerator compound No. | Concentration of accelerator in bleach-fix bath, mg./litre | Residual silver as percent of control |
|--------------------------|------------------------------------------------------------|---------------------------------------|
| 1                        | 100                                                        | 5.6                                   |
| 2                        | 150                                                        | 6.6                                   |
| 3                        | 100                                                        | 10.6                                  |
| 26                       | 150                                                        | 35                                    |
| 4                        | 150                                                        | 25                                    |
| 20                       | 150                                                        | 26                                    |
| 21                       | 100                                                        | 9.3                                   |
| 18                       | 150                                                        | 73                                    |

## Example 4

Pieces of the colour negative film were processed as follows:

|                    | Minutes |
|--------------------|---------|
| Colour developer B | 10      |
| Stop-fix           | 4       |
| Bleach-fix         | 16      |
| Wash               | 4       |
| Conditioner        | 4       |
| Wash               | 4       |
| Dry.               |         |

<sup>1</sup> With and without accelerator.

The silver content of the pieces of film was analysed with the following results:

TABLE 4

| Accelerator compound No. | Concentration of accelerator in bleach-fix bath, mg./litre | Residual silver as percent of control |
|--------------------------|------------------------------------------------------------|---------------------------------------|
| 1                        | 100                                                        | 11.2                                  |
| 21                       | 100                                                        | 20.9                                  |
| 18                       | 100                                                        | 65.4                                  |
| 19                       | 100                                                        | 33.8                                  |
| 23                       | 100                                                        | 46.1                                  |
| 14                       | 100                                                        | 71.4                                  |
| 15                       | 100                                                        | 52.2                                  |
| 16                       | 100                                                        | 93.6                                  |
| 5                        | 100                                                        | 36.8                                  |
| 6                        | 100                                                        | 11.5                                  |
| 17                       | 100                                                        | 60.6                                  |
| 24                       | 100                                                        | 90.6                                  |
| 25                       | 100                                                        | 84.5                                  |
| 11                       | 100                                                        | 56.4                                  |
| 8                        | 100                                                        | 31.2                                  |
| 9                        | 100                                                        | 38.2                                  |
| 7                        | 100                                                        | 29.5                                  |
| 10                       | 100                                                        | 35.3                                  |
| 22                       | 100                                                        | 24.2                                  |
| 12                       | 100                                                        | 66.5                                  |
| 13                       | 100                                                        | 89.9                                  |

## Example 5

A positive tripack colour material intended for the silver dye-bleach system comprising silver halide emulsions containing bleachable azo-dyes "Cibachrome" manufactured by Ciba-Geigy A.G. of Switzerland was given a neutral wedge exposure and processed, the processing sequence being as follows:

Development: 10 minutes

|                               |     |    |
|-------------------------------|-----|----|
| p-Methyl-aminophenol-sulphate | g-- | 1  |
| Sodium sulphite anhydrous     | g-- | 20 |
| Hydroquinone                  | g-- | 4  |
| Sodium carbonate anhydrous    | g-- | 10 |
| Potassium bromide             | g-- | 2  |
| Water to 1 litre.             |     |    |

Stop-fix: 4 minutes

|                                  |     |     |
|----------------------------------|-----|-----|
| Sodium thiosulphate pentahydrate | g-- | 200 |
| Sodium sulphite anhydrous        | g-- | 20  |
| Water to 1 litre.                |     |     |

Wash: 8 minutes

Dye-bleach: 20 minutes

|                                                                     |      |      |
|---------------------------------------------------------------------|------|------|
| Sulphuric acid, 96%                                                 | ml-- | 27.5 |
| Potassium iodide                                                    | g--  | 10   |
| Solution of 0.9 g. 2,3-dimethyl-6-aminquinoxaline in 50 ml. ethanol | ml-- | 15   |
| Water to 1 litre.                                                   |      |      |

Wash: 4 minutes

Bleach-fix: 6 minutes

|                                                            |      |      |
|------------------------------------------------------------|------|------|
| Disodium tetraborate decahydrate                           | g--  | 12.5 |
| Boric acid                                                 | g--  | 22.5 |
| Sodium hydroxide                                           | g--  | 10.0 |
| Ethylenediaminetetraacetic acid                            | g--  | 16.2 |
| Disodium salt of ethylenediaminetetraacetic acid dihydrate | g--  | 3.5  |
| Ferric chloride (60% w./v. solin.)                         | ml-- | 15   |
| Sodium thiosulphate pentahydrate                           | g--  | 95.0 |
| Sodium sulphite anhydrous                                  | g--  | 4.0  |
| Selenosemicarbazide                                        | mg-- | 100  |
| Water to 1 litre.                                          |      |      |

15 Wash: 8 minutes

Dry

The processed material was satisfactory and substantially no residual silver was left in the material even in the areas of high exposure. Similar silver-dye-bleach material was exposed and processed using the same solutions as set forth above except that the bleach-fix solution contained no selenosemicarbazide. Even when the material had been treated in the bleach-fix bath for 25 minutes it was unsatisfactory because it had a high minimal density due to 25 the incomplete removal of the residual silver in the areas of high exposure.

What we claim is:

1. In the processing of photographic material comprising exposed and developed silver halide emulsion 30 layers to yield material having colour dye images therein the step of treating the exposed and developed photographic material with a stable bleach-fix bath which comprises an aqueous solution of a mild oxidising agent which is strong enough to bleach the silver but not strong enough to oxidise silver halide solvents and a silver halide solvent which is either a water-soluble thiosulphate or a water-soluble thiocyanate in the presence of a bleach-fix 35 accelerator which is selected from (a) a water-soluble selenosemicarbazide of the general formula:



40 wherein one of  $R_1$  and  $R_2$  is a hydrogen atom or an alkyl, aralkyl or aryl group or a group  $R_6CO-$  where  $R_6$  is a hydrogen atom or an alkyl, alkoxy or heterocyclic group, or a group  $NR_7R_8-CSe-$  where  $R_7$  and  $R_8$  are each hydrogen atoms or alkyl groups and the other of  $R_1$  and

45  $R_2$  is a hydrogen atom or an alkyl group,  $R_3$  is a hydrogen atom or an alkyl, aralkyl or aryl group, one of  $R_4$  and  $R_5$  is a hydrogen atom or an alkyl, aralkyl or aryl group and the other of  $R_4$  and  $R_5$  is a hydrogen atom or an alkyl group, at least one of  $R_3$ ,  $R_4$  or  $R_5$  being a hydrogen atom and there being not more than one group selected from aryl, aralkyl and heterocyclic present in the compound or (b) a water-soluble compound of the general formula:



50 wherein each of  $R_9$ – $R_{16}$  is a hydrogen atom or an alkyl group there being not more than four alkyl substituent groups in the compound and at least one of  $R_9$ ,  $R_{10}$ ,  $R_{11}$ ,  $R_{14}$ ,  $R_{15}$ , and  $R_{16}$  being a hydrogen atom and  $X$  is a 55  $-(CH_2)_m-$

55 linkage group wherein  $m$  is 0 to 4, or (c) a water-soluble 1,2,4-triazole-3-solenol wherein the 5-carbon atom carries a substituent selected from a hydrogen atom or an alkyl, hydroxy, amino, alkylamino, arylamino or aralkylamino group and one of the nitrogen atoms carries a substituent selected from a hydrogen atom or an alkyl, aralkyl 60 or aryl group, or (d) a water-soluble 5,5-bis-1,2,4-tri-



azole-3-selenol wherein the triazole rings are linked directly or via a link

—(CH<sub>2</sub>)<sub>n</sub>—

wherein *n* is 1-4 and wherein one nitrogen atom in each of the triazole rings carries a substituent selected from a hydrogen atom and an alkyl, aryl and aralkyl group.

12. In the processing of exposed and developed photographic material comprising silver halide emulsion layers to yield material having colour dye images therein, the step of treating the exposed and developed photographic material with a stable bleach-fix bath which comprises an aqueous solution of a mild oxidising agent which is strong enough to bleach the silver but not strong enough to oxidise silver halide solvents and a silver halide solvent which is either a water-soluble thiosulphate or a water-soluble thiocyanate in the presence of a bleach-fix accelerator which is selected from the group consisting of

3-selenosemicarbazide;  
1-formyl-3-selenosemicarbazide;  
1-acetyl-3-selenosemicarbazide;  
1-propionyl-3-selenosemicarbazide;  
2-methyl-3-selenosemicarbazide;  
4-methyl-3-selenosemicarbazide;  
1,1'-dimethyl-3-selenosemicarbazide;  
1,2-dimethyl-3-selenosemicarbazide;  
1,2,4-trimethyl-3-selenosemicarbazide;  
1,1',4-trimethyl-3-selenosemicarbazide;  
1-acetyl-4-methyl-3-selenosemicarbazide;  
1-acetyl-4-benzyl-3-selenosemicarbazide;  
4-benzyl-3-selenosemicarbazide;  
1-phenyl-3-selenosemicarbazide;  
2-phenyl-3-selenosemicarbazide;  
4-phenyl-3-selenosemicarbazide;  
2-methyl-4-phenyl-3-selenosemicarbazide;  
1-(2-furoyl)-3-selenosemicarbazide;  
1,1'-oxalyl-bis (3-selenosemicarbazide);  
1,2,4-triazole-3-selenol;  
5-methyl-1,2,4-triazole-3-selenol;  
4,5-dimethyl-1,2,4-triazole-3-selenol;  
5,5'-bis(1,2,4-triazole-3-selenol);  
5,5'-methylene-bis(1,2,4-triazole-3-selenol);  
5,5'-ethylene-bis(1,2,4-triazole-3-selenol) and  
1-ethoxycarbonyl-3-selenosemicarbazide.

13. A process for the production of photographic material having colour dye images therein from exposed and developed photographic material comprising silver halide emulsion layers and including the step of treating the exposed and developed photographic material with a stable bleach-fix bath in the presence of a bleach-fix accelerator selected from the group consisting of

3-selenosemicarbazide;  
1-formyl-3-selenosemicarbazide;  
1-acetyl-3-selenosemicarbazide;  
1-propionyl-3-selenosemicarbazide;  
2-methyl-3-selenosemicarbazide;  
4-methyl-3-selenosemicarbazide;  
1,1'-dimethyl-3-selenosemicarbazide;  
1,2-dimethyl-3-selenosemicarbazide;  
1,2,4-trimethyl-3-selenosemicarbazide;  
1,1',4-trimethyl-3-selenosemicarbazide;  
1-acetyl-4-methyl-3-selenosemicarbazide;  
1-acetyl-4-benzyl-3-selenosemicarbazide;

- 14
- 4-benzyl-3-selenosemicarbazide;  
1-phenyl-3-selenosemicarbazide;  
2-phenyl-3-selenosemicarbazide;  
4-phenyl-3-selenosemicarbazide;  
5 2-methyl-4-phenyl-3-selenosemicarbazide;  
1-(2-furoyl)-3-selenosemicarbazide;  
1,1'-oxalyl-bis(3-selenosemicarbazide);  
1,2,4-triazole-3-selenol;  
5-methyl-1,2,4-triazole-3-selenol;  
10 4,5-dimethyl-1,2,4-triazole-3-selenol;  
5,5'-bis(1,2,4-triazole-3-selenol);  
5,5'-methylene-bis(1,2,4-triazole-3-selenol);  
5,5'-ethylene-bis(1,2,4-triazole-3-selenol) and  
1-ethoxycarbonyl-3-selenosemicarbazide.
- 15 14. A stable bleach-fix bath which comprises an aqueous solution of a mild oxidising agent which is strong enough to bleach the silver but not strong enough to oxidise silver halide solvents, a silver halide solvent which is either a water-soluble thiosulphate or a water-soluble thiocyanate and a bleach-fix accelerator which is selected from the group consisting of
- 20 3-selenosemicarbazide;  
1-formyl-3-selenosemicarbazide;  
1-acetyl-3-selenosemicarbazide;  
1-propionyl-3-selenosemicarbazide;  
2-methyl-3-selenosemicarbazide;  
4-methyl-3-selenosemicarbazide;  
1,1'-dimethyl-3-selenosemicarbazide;  
30 1,2-dimethyl-3-selenosemicarbazide;  
1,2,4-trimethyl-3-selenosemicarbazide;  
1,1',4-trimethyl-3-selenosemicarbazide;  
1-acetyl-4-methyl-3-selenosemicarbazide;  
1-acetyl-4-benzyl-3-selenosemicarbazide;  
40 4-benzyl-3-selenosemicarbazide;  
1-phenyl-3-selenosemicarbazide;  
2-phenyl-3-selenosemicarbazide;  
4-phenyl-3-selenosemicarbazide;  
2-methyl-4-phenyl-3-selenosemicarbazide;  
40 1-(2-furoyl)-3-selenosemicarbazide;  
1,1'-oxalyl-bis(3-selenosemicarbazide);  
1,2,4-triazole-3-selenol;  
5-methyl-1,2,4-triazole-3-selenol;  
4,5-dimethyl-1,2,4-triazole-3-selenol;  
45 5,5'-bis(1,2,4-triazole-3-selenol);  
5,5'-methylene-bis(1,2,4-triazole-3-selenol);  
5,5'-ethylene-bis(1,2,4-triazole-3-selenol) and  
1-ethoxycarbonyl-3-selenosemicarbazide.

#### References Cited

#### UNITED STATES PATENTS

|              |         |         |       |         |
|--------------|---------|---------|-------|---------|
| 2,131,038    | 9/1938  | Brooker | ----- | 96—109  |
| 2,410,690    | 11/1946 | Smith   | ----- | 96—66.3 |
| 55 3,396,017 | 8/1968  | Bacon   | ----- | 96—63   |
| 3,619,188    | 11/1971 | Alcock  | ----- | 96—60   |

NORMAN G. TORCHIN, Primary Examiner

J. R. HIGHTOWER, Assistant Examiner

60

U.S. CL. X.R.

96—60 R, 60 BF, 61 R, 62